

## UNITED STATES PATENT OFFICE

2,354,171

## LUBRICANT

John D. Morgan, South Orange, N. J., assignor to  
Cities Service Oil Company, New York, N. Y., a  
corporation of Pennsylvania

No Drawing. Application June 23, 1942,  
Serial No. 448,152

7 Claims. (Cl. 252—35)

This invention relates to lubricants. More particularly the invention relates to lubricants having a comparatively small change in viscosity over a wide temperature range.

The hydrocarbon lubricants which are made from petroleum, shales, and the hydrogenation of coal all have widely different viscosities over the temperature range which may be encountered in aviation, that is, from minus 40° F. to 200° F. It is desirable that products which have good lubricating properties should also have substantially uniform viscosities so that the lubricating qualities may be utilized at all of the various temperatures for which the lubricant is to be used.

I have discovered that the halogenated benzenes possess desirable lubricating characteristics and have to a large degree uniform viscosities over a wide range of temperatures. Many of the higher boiling halogenated benzenes are solid at temperatures between —40° and 200° F. On the other hand chlorbenzene has a melting point of —49° F., brombenzene a melting point of —23° F., and iodobenzene has a melting point of —19° F. Thus chlorbenzene is a fluid throughout the temperature range of —40° F. to 200° F. Chlorbenzene is soluble in practically all of the other halogenated benzenes so that it may be used to convert other halogenated benzenes from solid into lubricating fluids. By blending two or more of the halogenated benzene compounds together the mean boiling point of the mixture will be above the boiling point of the lower boiling point constituent and the vapor pressure of the mixture may be lowered considerably below the vapor pressure of the low boiling constituent.

The primary object of the present invention is to utilize the halogenated benzenes as lubricants.

A further object of the invention is to utilize a mixture of halogenated benzenes as a lubricant.

Another object of the invention is to utilize halogenated benzenes as lubricants and to utilize addition agents to inhibit the corrosion of metal bearing surfaces and to increase the lubricating and load-carrying qualities of the halogenated benzenes.

Another object of the invention is to utilize halogenated benzenes in the manufacture of lubricating greases.

A further object of the invention is to utilize the halogenated benzenes to produce a lubricating fluid which will have relatively uniform viscosity throughout the temperature range of —40° F. to 200° F.

With these and other objects in view the invention consists in the method of lubricating me-

tallic bearings and the lubricants therefor, which are hereinafter described and particularly defined in the claims.

The halogenated benzenes, such as the monohalogen benzenes, have comparatively high boiling points and comparatively low melting points. For example, chlorbenzene has a boiling point of 220° F. and a melting point of —40° F. Brombenzene has a boiling point of 388° F. and a melting point of —23° F. Iodobenzene has a boiling point of 371° F. and a melting point of —190 F. All of these monohalogen benzenes are mutually soluble.

Chlorination of the monohalogen compounds produces a series of dihalogen compounds and the chlorination of dihalogen compounds produces trihalogen compounds all of which have lubricating qualities and are comparatively high boiling constituents. Some of the halogenated benzenes having desirable lubricating qualities are:

|                       | Boiling point<br>° F. | Melting point<br>° F. |
|-----------------------|-----------------------|-----------------------|
| Orthodichlorbenzene   | 356                   | —                     |
| Paradichlorbenzene    | 344                   | 127                   |
| Orthodibrombenzene    | 435                   | 30                    |
| Metadibrombenzene     | 427                   | 34                    |
| Paradi brombenzene    | 426                   | 193                   |
| Orthodiiodobenzene    | 547                   | 80.6                  |
| Paradiiodobenzene     | 545                   | 265                   |
| Metadiiodobenzene     | 545                   | 104                   |
| 1,2,4-trichlorbenzene | 415                   | 61                    |
| 1,3,5-tribrombenzene  | 532                   | 247                   |
| 1,3,4-tribrombenzene  | 528                   | 111                   |

From the above table it will be seen that many of the polyhalogen benzenes are solid at ordinary atmospheric temperatures. Therefore if it is desired to produce a lubricating fluid such polyhalogen compounds must be diluted with the monohalogen compounds.

The dilution of the polyhalogen with the monohalogen compounds has advantageous properties because it tends to place the mean boiling point of the mixture considerably above the boiling point of the monohalogen and to place the vapor pressure of the mixture materially below the vapor pressure of the monohalogen. This is very desirable because the monohalogens as well as the polyhalogen compounds tend to volatilize at atmospheric pressure.

Furthermore it is desirable to use the halogenated benzene lubricants in closed bearings in order to minimize the volatilization of the halogenated benzenes.

Chlorbenzene has a comparatively flat viscosity curve or a comparatively uniform viscosity over

the temperature range of  $-40^{\circ}$  to  $200^{\circ}$  F. Chlorbenzene has the following viscosities:

| Temperature         | Viscosities in centistokes |
|---------------------|----------------------------|
| $-40^{\circ}$ F.    | 2.31                       |
| 0 <sup>o</sup> F.   | 1.67                       |
| 100 <sup>o</sup> F. | .64                        |
| 200 <sup>o</sup> F. | .47                        |

Dibrombenzene with one percent of Paraflo therein (chlorinated naphthalene) has the following viscosities:

| Temperature         | Viscosities in centistokes |
|---------------------|----------------------------|
| $-40^{\circ}$ F.    | 2.45                       |
| 0 <sup>o</sup> F.   | 1.46                       |
| 100 <sup>o</sup> F. | .67                        |
| 200 <sup>o</sup> F. | .46                        |

From this it will be seen that the monohalogen benzenes have a comparatively small change in viscosity over a wide temperature range.

Orthodichlorbenzene has a viscosity of .86 centistoke at  $100^{\circ}$  F. and .56 centistoke at  $200^{\circ}$  F. This product is solid at 0<sup>o</sup> F. and  $-40^{\circ}$  F. However, if 50 percent of chlorbenzene is dissolved in 50 percent of orthodichlorbenzene the blended mixture has a viscosity below 430 centistokes at minus  $30^{\circ}$  F. and less than 8 centistokes at  $100^{\circ}$  F.

1,2,4-trichlorbenzene, 1,3,4-trichlorbrombenzene and orthodibromobenzene may also be blended with chlorbenzene or brombenzene to produce fluid lubricants with advantageous viscosities at the lower temperatures. These compounds furthermore have comparatively high boiling points and are desirable for lubricating bearings at high temperatures.

The halogen benzenes may be compounded with metallic stearates for the production of greases. For example it has been found that orthodichlorbenzene, paradichlorbenzene, 1,2,4-trichlorbenzene, orthodibrombenzene, metadibrombenzene, and orthodibromobenzene may be dissolved in lithium stearate to produce lubricating grease. Preferably aluminum stearate is used with the lithium stearate as a blending agent to prevent the greases from bleeding. On the other hand all of these halogenbenzenes as well as chlorbenzene may be blended with calcium and sodium stearates to make greases. The blending of calcium and sodium stearates with the chlorbenzenes may be facilitated by a small amount of aluminum stearate.

An example of a lithium base grease is as follows:

|                                          | Percent by weight |
|------------------------------------------|-------------------|
| Chlorbenzene                             | 81                |
| Lithium stearate                         | 12                |
| Aluminum stearate                        | 6                 |
| Sulfurized tricresyl phosphate or Polane | 1                 |

Another example of a calcium base grease is as follows:

|                     | Percent by weight |
|---------------------|-------------------|
| Calcium stearate    | 10                |
| Aluminum stearate   | 6                 |
| Polane              | 1                 |
| Orthodichlorbenzene | 83                |
| 75                  |                   |

Another example of a sodium base grease is as follows:

|                                          | Percent by weight |
|------------------------------------------|-------------------|
| Sodium stearate                          | 13                |
| Aluminum stearate                        | 6                 |
| Sulfurized tricresyl phosphate or Polane | 1                 |
| Chlorbenzene                             | 80                |

Tests have been made on the mono- and polyhalogen benzenes and all of them exhibit good lubricating qualities. Furthermore if one percent of Polane, or one percent of sulfurized tricresyl phosphate is dissolved in these halogenated benzenes then such compounds have extreme pressure lubricating qualities. As shown in the examples above the extreme pressure addition agents are added to the greases in order to impart extreme pressure or high load-carrying characteristics to the greases.

The tricresyl phosphate mentioned herein is a sulfur condensed tricresyl phosphate or phosphite. This oil addition product is described in the patent to Engelke #2,260,303 granted October 28, 1941. This addition agent acts as an anti-corrosion agent, as well as an extreme pressure and oiliness agent.

The addition agent Polane, referred to above, is a commercial product on the market sold by the Patent Chemicals Company which is an ester of a fatty acid or a chlorinated ester of a fatty acid, such as chloromethyl stearate.

It will be apparent that blends of the monohalogen benzenes, which have the physical characteristics above-referred to, with the polyhalogen benzenes may be made to obtain substantially any desired characteristic of lubricant or grease. These benzene products are all simple compounds having definite characteristics and therefore have many advantages over lubricants which are made of a mixture of a large number of hydrocarbons having different physical and chemical characteristics. Furthermore, the blending of the various halogenated benzenes can be readily worked out on account of the fact that pure compounds may be used in making simple mixtures.

The preferred form of the invention having been thus described, what is claimed as new is:

1. A lubricant comprising a halogenated benzene with a small amount of an inhibitor comprising a chlorinated ester of a saturated higher fatty acid.

2. A lubricant comprising a mixture of halogenated benzenes which are inhibited against corrosion of metal bearings with a small amount of chlorinated ester of a saturated higher fatty acid.

3. A lubricant comprising:

|                       | Percent by weight |
|-----------------------|-------------------|
| Chlorbenzene          | 81                |
| Lithium stearate      | 12                |
| Aluminum stearate     | 6                 |
| Chloromethyl stearate | 1                 |

4. A lubricant comprising:

|                       | Percent by weight |
|-----------------------|-------------------|
| Sodium stearate       | 13                |
| Aluminum stearate     | 6                 |
| Chloromethyl stearate | 1                 |
| Chlorbenzene          | 80                |

5. A lubricant consisting essentially of a chlorinated benzene inhibited against corrosion and reinforced for load carrying capacity with small

amounts of a corrosion inhibitor and an extreme pressure addition agent.

6. A lubricant comprising a halogenated benzene having a metallic stearate dissolved therein and inhibited against corrosion by a chloromethyl stearate.

7. A lubricating grease comprising approximately 80% of a chlorbenzene in which is dis-

solved a mixture of metal stearates in sufficient amount to impart a grease consistency, said grease being inhibited against corrosion and reinforced for load-carrying capacity with small amounts of a corrosion inhibitor and an extreme pressure addition agent.

JOHN D. MORGAN.